

## UNITED STATES PATENT OFFICE

2,099,190

## PROCESS FOR DEWAXING OILS

Charles Douglas Barnes, Long Beach, and Marcellus T. Flaxman, Wilmington, Calif., assignors to Union Oil Company of California, Los Angeles, Calif., a corporation of California

No Drawing. Application February 24, 1936,  
Serial No. 65,414

10 Claims. (Cl. 196—19)

The present invention relates to improvements in the art of separating wax from wax-bearing oil, such as lubricating oil distillates or residues. More particularly, the invention pertains to a method in which certain materials are added to the wax-bearing oil to condition it so that the wax may be more readily separated from the oil. This invention is also applicable to a process for the separation of oil from waxes, such as slack 5 wax, wax cakes, etc.

Many lubricating oil fractions contain relatively large quantities of wax which impart a high pour point to the oil and thereby render these oils less desirable as motor lubricants as they are 10 solid and will not flow at ordinary temperatures. In order to make these oils suitable for use at ordinary temperatures, it is necessary to remove the wax contained in the oil. This is usually accomplished by adding a suitable diluent to the 15 wax-bearing oil, chilling the diluted oil to a temperature sufficiently low to congeal the wax content and then removing the wax from the diluted oil by settling, centrifuging, or filtering.

It is well known that an efficient dewaxing 20 process is one in which the wax may be removed as rapidly as is possible to produce a large amount of dewaxed oil having a reasonably low pour point and to produce a wax reasonably free from oil, that is, having a high melting point. In other 25 words, it is desirable to separate the wax from the oil, for example, by filtration, at a very high rate and yet to recover as much wax-free oil as is possible from the original stock. In many of the 30 processes now in use, it is possible to produce oils of low pour point; however, the yield of oil recovered is unsatisfactorily low and the melting point of the separated wax is low, indicating that a large amount of oil is retained in the wax. Also, the rate at which the wax is separated from 35 the oil by filtration, for example, is also low.

We have discovered that the wax contained in 40 oils may be more readily separated by mixing the wax-bearing oil with certain materials which render the wax more readily separable from the oil. Hereinafter, the materials which we desire to employ to condition the wax present in the wax-bearing oil in order to effect more ready separation of the wax from the oil will be referred to as "wax separation aids".

45 We have discovered wool grease and lanolin to be quite effective as wax separation aids in the dewaxing of waxy oils. We have further discovered that oxidized wool grease and oxidized lanolin to be even more effective as wax separation aids than the unoxidized materials. The

reason for the unexpected activity of the aforementioned wax separation aids in dewaxing oils is not definitely known but it is known that when a small amount of either the oxidized or unoxidized material is added to the oil to be dewaxed, 5 an improvement is obtained with respect to the yield of dewaxed oil, filter rate, and melting point of the separated wax as compared to similar dewaxing conditions when no wax separation aid is employed. One explanation for this phenomenon 10 may be that since the aforementioned wax separation aids contain material amounts of cholesterol and derivatives related to cholesterol, it is possible that such ingredients are largely 15 responsible for the potency of the aforementioned wax separation aids.

Wool grease, as is well known, is the grease which naturally protects the wool while on sheep or other animals and which amounts to about 20% of the fleece. This may be removed from the 20 fleece by scouring the fleece with a detergent solution such as, for example, a soap and sodium carbonate solution or by other means utilizing a hydrocarbon solvent such as a high test gasoline or naphtha which has no effect upon the wool. 25 In the latter case, the solution of naphtha and grease is run into a still whereupon the greasy solvent is heated to drive off the gasoline or naphtha. The grease which remains in the still is washed with warm water and dried by blowing 30 with warm air. Wool grease is sometimes referred to in the United States as degras. The following are the approximate characteristics of wool grease as recovered by the aforementioned process:

|                                         |                |    |
|-----------------------------------------|----------------|----|
| Melting point                           | 97 to 108° F.  | 35 |
| Moisture content                        | 2 to 2½%       |    |
| Ash                                     | 0.1 to 0.8%    |    |
| Free fatty acid (figured as oleic acid) | about 9 to 10% | 40 |
| Saponifiable matter                     | about 60%      |    |
| Specific gravity at 60° F.              | .967           |    |
| Saponification number                   | 113 to 123     |    |
| Acid value                              | not over 20.9% |    |
| Viscosity at 210° (Tagliabue)           | 284 to 292     | 45 |
| Flash point                             | 372 to 390° F. |    |
| Fire test                               | 527 to 536° F. |    |
| Cold test                               | 94° F.         |    |
| Iodine value                            | about 27       | 50 |

In general, the oxidized wax separation aids may be produced by subjecting the unoxidized materials aforementioned to the action of an oxygen containing gas, such as air, oxygen, ozone or hydrogen peroxide, preferably at elevated tem- 55

perature. Certain of the materials among those mentioned above, require no further treatment, chemical or otherwise previous to oxidation to produce the active wax separation aid. However, 5 in the case of wool grease, it is preferable to dehydrate the material prior to oxidation.

The wool grease either chemically treated or dehydrated, as the case may be, is then subjected to oxidation. The conditions and degree of oxidation will vary with the type of material treated. 10 The oxidation consists in heating the wool grease, for example, to a temperature of about 350° F. and introducing air, oxygen, ozone or hydrogen peroxide into the charge until sufficient oxidation 15 has taken place to render the material active as a wax separation aid and yet retain its compatibility with the oil to be dewaxed. In one case, oxidation of wool grease was effected by introducing air while maintaining the charge at 20 about 340° F. for a period of about 200 hours.

The oxidation reaction with air, oxygen or ozone, or with hydrogen peroxide, may be aided when the oxidation reaction is carried out in the presence of catalysts. Catalysts which may 25 be employed with benefit for this purpose are metal chlorides, such as the chlorides of iron, zinc, tin, aluminum, metal soaps, such as the naphthenates, oleates, stearates, ricinoleates, palmitates of sodium, copper, magnesium, aluminum, cobalt, and iron.

In carrying out the dewaxing process, a small amount, i. e. 0.3% to 1% by volume of the oxidized or unoxidized wax separation aid is mixed with or dissolved in the wax-bearing oil, 30 after which the mixture is chilled to a sufficiently low temperature to precipitate or solidify the wax contained in the oil. The solidified wax may then be separated from the chilled mixture by settling, centrifuging, or filtering. The added 35 wax separation aid will be precipitated and removed along with the wax. If desired, a concentrated oil solution of the wax separation aid may be produced by first mixing or dissolving a small quantity of the waxy distillate to be dewaxed with the wax separation aid at an elevated temperature, such as, for example, about 40 350° F. The concentrated solution may then be added to the waxy distillate in an amount as to incorporate the desired amount of the wax separation aid into the oil to be dewaxed.

In many cases, it is desirable to dilute the mixture of wax-bearing oil and wax separation aid with a suitable diluent prior to the chilling step in order to render the oil fluent at the dewaxing 45 temperature. As diluents, we preferably employ liquefied normally gaseous hydrocarbon such as ethane, ethylene, propane, propylene, butane, butylene, or mixtures thereof or we may employ such light hydrocarbons such as pentane, hexane, heptane, octane, nonane, or hydrocarbon fractions, such as naphtha, gasoline, kerosene, or gas oil. We may also employ such diluents as acetone, mixtures of acetone and benzol, ethyl, propyl and butyl alcohols, methyl ethyl ketone, diethyl ketone, methyl propyl ketone, ethyl propyl ketone, cyclo hexanone, normally gaseous and normally liquid ethers, methyl chloride, dichlorethylene, or trichlorethylene, or mixtures of these hydrocarbons with the aforementioned 50 hydrocarbons.

The use of a liquefied normally gaseous diluent, such as liquid propane, is preferred, since in addition to having the property of retaining less wax in solution at low temperatures, it may 55 be employed to produce the necessary degree of

refrigeration to precipitate the wax from the solution by vaporizing a portion of the liquefied normally gaseous material from the diluted oil under reduced pressure.

It is thus an object of our invention to improve dewaxing characteristics of wax-containing oil by adding a small quantity of an oxidized or unoxidized wool grease or lanolin to the oil to be dewaxed. 5

A further object of our invention resides in 10 dissolving the wax-bearing oil to be dewaxed and the aforementioned wax separation aid in a suitable diluent, chilling the mixture to congeal the wax content and separating the congealed wax and oxidized wax separation aid from the diluted 15 oil by filtration, centrifuging or settling.

Many specific objects, features and advantages of our invention will become apparent to those skilled in the art as the description of our invention proceeds in connection with the specific 20 examples given below which are not to be considered as limiting our invention but merely 25 illustrative of methods of carrying it out.

In one run, about 350 grams of the wool grease 30 having the characteristics aforementioned was heated in a still to a temperature of about 200° F. and was blown gently with air until approximately the entire moisture content was distilled from the material. Thereupon, the temperature was increased to approximately 340° F. and was 35 maintained at such temperature for approximately 200 hours during which time air was introduced into the charge at a rate of approximately 10 liters per hour. This resulted in the production of an oxidized wool grease which had 40 the following characteristics:

|                       |          |
|-----------------------|----------|
| Acid number           | 23.0     |
| Saponification number | 147      |
| Gravity at 60° F.     | 0.991 40 |

The oxidized wool grease was mixed in a closed vessel with an SAE 20 waxy lubricating oil distillate obtained by the vacuum distillation of a Santa Fe Springs crude oil. The admixture was accomplished at a temperature of about 300° F. 45 and in an amount as to incorporate approximately 0.5% by weight into the waxy distillate. The resultant mixture was then diluted with approximately 3.0 volumes of liquid propane under super-atmospheric pressure to one of the oil 50 containing the wax separation aid. The temperature of the resultant mixture was about 130° F. and the pressure was about 250 lbs. per square inch. The mixture of waxy lubricating oil, propane, and oxidized wool grease was then chilled 55 externally at a rate of approximately 3° F. per minute until a temperature of approximately -40° F. was attained, the refrigeration being accomplished by vaporizing under gradually reduced pressure a portion of propane in a jacket surrounding the chilling vessel. The chilled slurry of propane, lubricating oil and solidified wax and wax modifier was then filtered under a pressure of approximately 25 lbs. per square 60 inch in order to effect the separation of the precipitated wax and wax modifier from the chilled propane solution of lubricating oil. The filter rate was approximately 16.6 gallons per square foot of filter surface per hour based on propane 65 free oil. After distilling the filtrate in order to remove propane, a yield of approximately 84.0% by volume of dewaxed oil was recovered having a pour point of 5° F. The separated wax had a melting point of about 127° F. as determined by the Ubbelohde method. 70 75

The results obtained in the foregoing example indicate that this type of wax separation aid is quite active in dewaxing oils when it is compared with a blank run wherein no wax separation aid is employed. A blank run on the same oil using the same amount of propane and carried out under the same conditions as above, showed that only approximately 64.8% by volume of oil was obtained having a pour point of 10° F. The wax separated from the oil had a melting point of only 117° F. The filter rate was only 2.4 gallons per square foot per hour.

In another run, unoxidized dehydrated wool grease was substituted for the oxidized wool grease in the above example. The results obtained indicate that this wax separation aid while not quite as potent as the oxidized material was sufficiently effective to warrant its use in commercial dewaxing processes. In this run, the filter rate was approximately 11.5 gallons per square foot per hour; the yield of dewaxed oil was 79.6% by volume with a pour point of 10° F. while the separated wax had a melting point of about 126° F.

Another run similar to the above but substituting oxidized lanolin which is a highly refined wool grease showed results as follows: The filter rate was approximately 19.3 gallons per square foot per hour; the yield of dewaxed oil was 82.2% by volume having a pour point of 5° F. and the melting point of the separated wax was about 127° F.

It will be observed that the foregoing description of our invention is not to be considered as limiting as many variations thereof may be made by those skilled in the art within the scope of the following claims.

We claim:

1. A process for conditioning oils preparatory to the separation of wax therefrom which comprises mixing said wax and oil with a wax separation aid containing cholesterol. 5
2. A process for separating wax from wax-oil mixtures which comprises mixing the wax-oil mixture with a wax separation aid containing cholesterol, chilling the mixture to solidify the wax content and separating the solidified wax from the oil. 10
3. A process for separating wax from wax-oil mixtures which comprises mixing the wax-oil mixture with a wax separation aid containing cholesterol and a diluent, chilling the mixture to 15 solidify the wax content and separating the solidified wax from the oil.
4. A process as in claim 2 in which the wax separation aid comprises wool grease. 20
5. A process as in claim 2 in which the wax separation aid comprises lanolin. 25
6. A process as in claim 3 in which the diluent comprises a liquefied normally gaseous hydrocarbon.
7. A process as in claim 3 in which the wax separation aid comprises wool grease. 30
8. A process as in claim 3 in which the wax separation aid comprises lanolin.
9. A process as in claim 3 in which the wax separation aid comprises wool grease and the diluent comprises a liquefied normally gaseous hydrocarbon. 35
10. A process as in claim 3 in which the wax separation aid comprises lanolin and the diluent comprises a liquefied normally gaseous hydrocarbon.

CHARLES DOUGLAS BARNES.  
MARCELLUS T. FLAXMAN.